

1

3,226,321

**SOLIDS HAVING IMPROVED ELECTRICAL CONDUCTIVITY**

John P. McDermott, San Diego, Calif., assignor to Esso Research and Engineering Company, a corporation of Delaware  
No Drawing. Filed Dec. 17, 1962, Ser. No. 244,874  
7 Claims. (Cl. 252—8.8)

This application is a continuation-in-part of pending application Serial Number 82,692, filed January 16, 1961.

The present invention relates to the use of organic phytates and particularly to the use of organic nitrogen base phytates to improve the electrical properties of solid materials which have a tendency to generate, accumulate, or retain electrical charges.

There has been a growing need and urgency for effective materials to aid in improving the electrical properties of nonconductive solid materials that have a tendency to generate, accumulate or retain electrical charges on their surfaces. In particular, the generation and/or accumulation of electrical charges on hydrophobic nonconductive materials such as synthetic materials, plastics, resins, rubbers, and textile fibers has been a vexing problem. The quantity and seriousness of the charges depend in part upon the nature of the material, the temperature, humidity, and the like. The hydrophobic nature of synthetic fabrics and textiles or their blends with natural animal and vegetable fibers and materials has hampered their effectiveness and full commercial use. The tendency of these synthetic textiles to generate and accumulate electrical charges renders their handling and processing hazardous by virtue of the danger of electrical discharges. Further, electrical charges accumulated on these materials have a pronounced tendency to attract dust and other deleterious material having an opposite charge.

Attempts to remedy and rectify the foregoing problem have prompted the use of radioactive metal bars to neutralize the charge by ionizing the atmosphere near the charged surface, by the use of conductive copper tinsel or other grounding means in contact with the charged surface, and the like. The subsequent employment of synthetic materials as textile fabrics has resulted in the well known "clinging" effect by virtue of the static charges on the materials. This clinging effect is particularly noticeable on the human body after certain motion has generated a charge on the fabric surface or by the attraction of other materials after a synthetic fabric has been tumbled, such as in a dryer. Attempts to solve this problem have utilized certain additives on the surface of the fabric or material to promote electrical conductivity, and thus aid in dissipating the charge before an excessive charge is allowed to accumulate. These additives have not proven to be entirely satisfactory or practical in that some are readily susceptible to removal on laundering of the fabric or on contact with water, or alter the feel or surface of the fabric and the like.

It is an object of this invention to provide a class of additives which effectively dissipate electrical charges generated on solid materials such as fabrics.

The object of this invention is attained through the use of organic phytates, particularly organic nitrogen base phytates, and preferably organic ammonium phytates. These materials may be described more specifically as hydrocarbyl ammonium phytates. These phytates are formed by the reaction of an acidic phytate with a basic organic nitrogen compound to yield an organic nitrogen base phytate. The nitrogen base radical comprises a nitrogen atom having four substituent groups, at least one group being an organic radical with the ammonium nitrogen atom substituent groups being selected from the class

2

consisting of hydrogen and organic radicals. The organic radicals are preferably directly bonded to the nitrogen atom by a carbon atom of an organic radical, and especially an organic radical having from 1 to about 30 carbon atoms.

The aliphatic ammonium phytates are the preferred materials of the invention with the oil soluble tertiary ammonium phytates particularly preferred, while a mixed tertiary and quaternary ammonium phytate prepared by the neutralization of phytic acid with a tertiary amine and a quaternary ammonium hydroxide mixture being especially preferred.

The organic nitrogen base phytates of the invention may be prepared by reacting phytic acid or an acidic phytate salt such as calcium phytate or ammonium phytate, or an acidic partial ester or acidic metal phytate complexes, such as alkaline earth or heavy metal complexes, and the like, or preferably phytic acid with a basic organic nitrogen base compound. The preferred method of preparation is the reaction of phytic acid with a basic amine or a quaternary ammonium compound. The resulting water from the reaction or from the phytic acid concentrate may be removed by means of an azeotropic distillation employing an organic solvent such as benzene, toluene, hexane and the like. The reaction of phytic acid and a quaternary ammonium compound is an acid base type of displacement reaction. Thus, the reaction of phytic acid with quaternary ammonium hydroxide yields the desired quaternary ammonium phytate and water of the reaction. The reaction of phytic acid and an amine is an addition type of reaction with theoretically no by-product of the reaction obtained. Both reactions will yield the nitrogen base organic ammonium phytates of the invention. The organic ammonium phytates of the invention are believed to be phytates composed of a positively charged nitrogen base cation and a negatively charged phytate anion. The number of cations in the molecule may be varied from 1 to 12, depending upon the number of acidic hydrogen atoms removed from the acidic phytate anion.

The ratio of the acidic phytate to the basic organic nitrogen compound, e.g. phytic acid to quaternary ammonium hydroxide or amine, may be varied widely. Depending upon the ratio of the reactants employed, the organic phytate salt formed may have from 1 to 12 basic ammonium radicals. In general, it has been found that the salts containing from about 1 to about 6 quaternary ammonium groups are somewhat more effective than the more fully substituted salts. The use of the mono-substituted to hexa-substituted phytate compounds for promoting electrical conductivity is therefore preferred.

The quaternary ammonium hydroxides which are employed in preparing the quaternary ammonium phytates include those hydroxides wherein organic radicals attached to the central ammonium nitrogen atom may be substituted or unsubstituted, aliphatic, alicyclic, heterocyclic, aromatic, or arene radicals, including alkylaryl and arylalkyl, of from 1 to about 30 carbon atoms, or combinations thereof. These organic radicals may have substituent groups such as hydroxyl, sulfhydryl, halogen, ether bound oxygen, acetylenic groups, nitro, sulfur, sulfoxyl, and the like. Due to economic availability, present cost, and electrical characteristics, the tetra-aliphatic quaternary ammonium hydroxides are the preferred reactants of the quaternary ammonium hydroxides. The substituent groups may be alkyl, alkenyl, alkynyl, cycloalkane, and cycloalkene radicals of from 1 to 30 carbon atoms, or combinations thereof.

Examples of suitable quaternary ammonium phytates prepared by reacting phytic acid with quaternary ammonium hydroxide include tetramethyl ammonium phytates, tetrapropyl ammonium phytates, methyltributyl

ammonium phytates, dimethyldibutetyl ammonium phytates, isopropyltriethyl ammonium phytates, diethyl dihexadecyl ammonium phytates, dimethyldioleyl ammonium phytates, trimethyloleyl ammonium phytates, butyl-trioleyl ammonium phytates, dibutyldicyclopentyl ammonium phytates, tetraheptadecyl ammonium phytates, tetraicosyl ammonium phytates, dimethyl benzyl soya ammonium phytates, triethyltolyl ammonium phytates, trimethylcyclohexyl ammonium phytates, octadecyl-dimethyl benzyl ammonium phytates, 1-ethylquinolinium phytates, trimethylphenyl ammonium phytates, 1-ethyl-pyridinium phytates, cetyltrimethyl benzyl ammonium phytates, tributyl-4-octynyl phytates, dimethylpropyl-4-nitrooctyl phytates, trimethyl-10-mercaptooctadecyl ammonium phytates, dimethyl-di-(10-chlorooctadecyl) ammonium phytates, and the like.

All of the above salts may contain from 1 to 12 ammonium groups. The especially preferred quaternary ammonium phytates are those oil soluble phytates having a mixture of lower alkyl groups and aliphatic groups of from 8 to 18 carbon atoms, such as dialkyl dialiphatic C<sub>8</sub>-C<sub>18</sub> phytates, wherein the aliphatic groups are derived from commercially available saturated and unsaturated fatty acid radicals. The basic nitrogen compounds useful in the preparation of the compounds may also include nitrogen compounds having substituent groups derived from naturally occurring materials such as from vegetables, animal and marine fats and oils like beef tallow, soybean, coconut, cottonseed, olive, linseed, palm kernel, corn, peanut, cod, whale, tung, lard, and the like. These fats and oils are mixtures of saturated and unsaturated enoic dienoic and dienoic fatty acids of from about 8 to 20 carbon atoms per molecule. Quaternary ammonium compounds and amines suitable for preparing the inventive phytates and containing fatty acid substituent groups as above are available from commercial sources. An example of a suitable commercial tertiary amine is a methyl disoja amine wherein the soya radical contains approximately 20 weight percent hexadecyl, 17 weight percent octadecyl, 26 weight percent octadecenyl, 37 weight percent octadecadienyl and about 7 weight percent of other unidentified material. Suitable commercial amines include those with a mean molecular weight of from 260 to about 530. Tertiary aliphatic amines having one lower alkyl group of from 1 to 6 carbon atoms and at least one long chain aliphatic group of from 8 to 18 carbon atoms, e.g. derived from fatty acids, yield particularly effective oil soluble aliphatic tertiary ammonium phytates. Commercial amines would thus include methyl dioleyl amines, methyl dihydrogenated tallow amines, dimethyl soya amine, ethyl disoja amine, methyloleyl amine, ethyl soya amine, dimethyl coco amine, and the like.

A suitable commercial quaternary ammonium hydroxide whose substituent groups are derived from naturally occurring materials would be trimethyl soya ammonium hydroxide, dimethyl dicoco ammonium hydroxide, dimethyl ditallow ammonium hydroxide and the like. Quaternary ammonium compounds and amines having one and preferably two or more of such naturally occurring fatty acid groups are generally less expensive and readily available and therefore commercially preferred for preparing oil soluble phytates.

The basic organic nitrogen radical of the ammonium phytates may also be derived from the reaction of an acid phytate, such as phytic acid, or a partially neutralized phytate, with a substituted or unsubstituted primary, secondary, or tertiary organic amine; diamines; polyamines; hydroxyl amines; carboxylic amines; amidines; and the like. The amines may have substituted or unsubstituted, aliphatic, alicyclic, aromatic heterocyclic, or arene organic radicals of from 1 to 30 carbon atoms or combinations thereof. Aliphatic amines, such as unsubstituted aliphatic amines having alkyl, alkenyl, and alkynyl radicals and mixtures thereof, and especially oil soluble tertiary aliphatic amines, are preferred materials.

Suitable amines include primary amines such as p,p'-dibutyldiphenyl amine, 4-amin- $\alpha$ -naphthyl amine, ethyl amine, sec butyl amine, allyl amine, 2-amino ethanol, 2-phenyl ethyl amine,  $\alpha$ -methyl benzyl amine, 2-amino-2-methyl-1-propanol, para-amino benzoic acid, toluidine, chloroaniline, urea, thiourea, octylamine, oleylamine, cyclohexylamine, benzylamine, p-methoxybenzylamine, p-anisidine, aniline, 1-naphthylamine, p-aminophenol, octyl-p-aminobenzoate, p-octylaniline, and the like; secondary amines such as: di-isoamylamine, di-oleylamine, di-soya amine, di-cyclohexylamine, N-methylcyclohexylamine, di-phenylamine, N-octyl-1-naphthylamine, N,N'-bis-(t-octyl)thiourea, N-phenyl-N'-t-octylurea, N-octylcyclohexylamine, N-(2-ethylhexyl)aniline, quinoline morpholine and alkyl morpholine, such as N-methyl and N-ethyl morpholine, phenothiazine, dimethylpiperidine, piperidine, pyrrolidine, dihydrogenated tallow amine, pyrazole, pyrazoline, p-methylaminophenol, and the like; tertiary amines such as: tributyl amine, methyldisoya amine, methyldioleylamine, dimethyloleylamine, 2-diethylamino ethanol, tribenzylamine, N,N-dibutylcyclohexylamine, N,N-dibutylaniline, di(2-ethylhexyl)ethanolamine, N-dodecylmorpholine, pyridine,  $\beta$ -picoline, pyrazine trioleylamine, N-octyl cyclohexyl amine, N-methyl-2-pyrrolidone, polyvinyl pyrrolidone, and the like; alkaloids such as: nicotine, morphine, quinine, papaverine, ephedrine, tropine, atropine, coniine, cocaine, brucine, and the like; polyamines, including diamines and diamino dialkyl amines such as: hexamethylene-tetramine, ethylene diamine, 1,6-hexanediamine, p-phenylenediamine, N-oleylpropane diamine-1,3 piperazine, N,N'-dibutyl-p-phenylenediamine, tetramethylethylene diamine, dimethylaminomethyl phenols, triamines like aminoethyl piperazine, combining a primary, secondary, and tertiary amine group in a single molecule, and the like; carboxylic amines or amino acids such as: aminoacetic acid, p-aminophenylacetic acid, 4-aminobutyric acid, 2-amino hexanoic acid, and the like; azo amines such as: p-dimethylaminoazobenzene-o-carboxylic acid, azobenzene, p-phenylazobenzene, and the like; guanidines and amidines such as: p-butylphenyl guanidine, phenyl biguanidine, benzoguanamine, triphenyl guanidine, 1,3-di-o-tolyl guanidine, tetramethyl guanidine, formamidine, N,N-diphenyl formamidine, and the like; hydrazines such as: alkyl hydrazine, aryl hydrazine and quaternary hydrazinium bases, hydrazine, phenylhydrazine, N,N-dimethyl-N-octadecylhydrazinium hydroxide, dimethyl hydrazine, and the like; hydroxyl amines or amino alcohols such as: alkanol amines, triethanol amines, 3-diethyl amino-1-propanol, 2-amino ethanol, 1-amino-2-propanol, 2-2'-imino diethanol, 2-amino-2-methyl-1,3-propane diol, 2-anilinoethanol, t-butyl amino ethanol, the alkyl alkanol amines like methyl ethanolamine, ethyl ethanolamine, ethyl diethanolamine, and the like; polyalkoxyl amines such as tripolyethoxy amine and the like.

It is seen that the preferred ammonium and amine compounds of this invention have a C:N atomic ratio greater than 2/1, and preferably at least 3/1. These ammonium and amine compounds are most effective when reacted with the phytic acid in reducing electrical charge of the solid materials.

Phytic acid, the preferred reactant material to form the organic phytates of this invention is the hexaphosphoric acid ester of inositol. This compound has the formula:



Those organic ammonium phytates wherein the organic nitrogen base is a mixture of an aliphatic quaternary ammonium hydroxide and a tertiary aliphatic amine and particularly those having a quaternary to amine ratio of between 4:1 and 1:4, and preferably 3:1 to 1:1, are especially preferred additives. For example, phytic acid may be neutralized with a mixture of a dimethyldioleyl ammonium hydroxide and a methyl disoya amine to yield an effective mixture of ammonium phytates.

The organic nitrogen base phytates of the invention are profitably employed in treating nonconductive solid material such as paper, rubber, plastics, resins, asbestos, wood, and synthetic fibers and textiles, and blends thereof in order to promote the electrical conductivity of the surface. The textile fibers or other materials may be treated with the inventive phytates by brush, spray, dip, coating, impregnation, or other convenient means or techniques of application for treating the surface of the material to be protected with the desired phytate. The treated material may be synthetic plastics and resins in fiber, fabric, film, tube, or other form. Suitable synthetic textile fibers which would be benefited by treatment with the phytates of the invention include arcylics, polyesters, polyamides, polyethylene, polypropylene, polyvinyl chloride, glass fibers, and the like, and blends thereof with other materials such as wool, cotton, felt, asbestos, and other ingredients. The phytate treatment may be beneficially accomplished in the presence or absence of other finishing and testing materials, such as starch, wrinkle-proofing ingredients, resin finishes, and the like.

The organic ammonium phytates may be successfully employed by treating the desired material so as to deposit a minor amount of the phytate on the surface to be protected. Preferred methods of application include dipping or impregnating the item to be treated in a solution of a volatile liquid solvent such as an aliphatic or aromatic alcohol like benzyl alcohol, isopropanol, ethanol; an ether anisole, ethyl ether; a hydrocarbon like toluene, heptane; a halogenated solvent like chloroform, perchloroethylene and the like; or combinations thereof which may contain from 0.1 to 10.0 weight percent of the desired additive and usually from 0.5 to 2.0 weight percent. In certain cases, direct contact by wiping the phytate directly or in admixture with paraffin or other filler materials directly on the surface is recommended.

The exact nature and objects of the invention may be more fully understood from the following examples.

#### Example 1

Quaternary ammonium salts of phytic acid were prepared by reacting dimethyldioleyl ammonium hydroxide with phytic acid in varying amounts.

The quaternary ammonium hydroxide was added to a mixture of phytic acid in benzene, with stirring, in a flask equipped with a condenser and water trap. After addition was complete, the reaction mixture was distilled until all the water was removed. The products, obtained on evaporation of the benzene, were cream-colored, waxy solids. Analysis showed the salts prepared to be mono-dimethyldioleyl ammonium phytate, tri-dimethyldioleyl ammonium phytate, hexa-dimethyldioleyl ammonium phytate and dodecyl-dimethyldioleyl ammonium phytate. Other quaternary ammonium phytates of the examples were prepared in a similar manner and also mono-tetradecyl ammonium phytate.

#### Example 2

Other organic ammonium phytates were prepared by reacting a tertiary aliphatic amine such as methyl disoya amine with phytic acid in varying amounts.

The mono-methyl disoya ammonium phytate was prepared by adding ten grams (about 0.014 mole active ingredient) of a methyl disoya amine commercial mixture to a stirred dispersion of 13.2 grams (0.014 mole) of phytic acid (70% solution in water) in benzene-xylene,

followed by azeotropic distillation to remove the water. Subsequent filtration of the slightly hazy reaction mixture yielded a clear concentrate of the mono-methyldisoya ammonium phytate in xylene in approximately theoretical yield amounts. The mono-methyldisoya amine phytate will be hereafter identified as mono M2SA phytate. Other amine salts, as in the examples, were prepared in a similar manner; and also prepared in this manner were mono-soya ammonium phytate, hexa-soya ammonium phytate, di-diethanol soya ammonium phytate, and di-dimethyl soya ammonium phytate.

#### Example 3

The ammonium phytates of the invention have been discovered to be effective in promoting the electrical conductivity on the surfaces of solid materials such as nonconductive synthetic textiles, plastics, and the like. When employed in treating the surface of a nonconductive material, such as a textile fabric, the ammonium phytates do not alter the appearance or feel of the treated surface and further are resistant to removal by laundering with aqueous detergents and soap, water contact, and dry cleaning solvents. The ammonium phytates may be applied by dipping the item to be tested into a solution of the phytate in a volatile solvent followed by evaporation of the solvent, or may be applied by wiping the pure additive material directly on the surface to be tested, or by spraying from an aerosol can, or other convenient methods of application.

To demonstrate the efficacy of the ammonium phytates in preventing static generation arising from the frictional contact of solid surfaces, such as textiles, plastics, rubber, and the like, a test was performed utilizing the Keithley electrometer. This instrument (Model 200) was equipped with a Keithley static detector (Model 2005). The test materials used were twelve-inch square pieces of nylon jersey cloth.

A piece of cloth was stroked several times with Lucite rod. When the cloth was placed near the static detector, the meter needle jumped beyond the 10 volt meter scale in the negative direction; when the Lucite rod was placed near the static detector, the needle jumped off-scale in the opposite direction.

#### Example 4

The cloth, treated as described in Example 3, was dipped in a 1.0% solution of di-dimethyldioleylammonium phytate in chloroform. After evaporation of solvent the above test was repeated. This treated cloth showed no activity—the meter needle remained at zero. The Lucite rod, however, was still active.

#### Example 5

A small amount of the pure dimethyldioleylammonium phytate (solvent-free) was rubbed on the Lucite rod of Example 4 after which it was wiped with a clean cloth. The treated rod showed no static activity after contact with untreated cloth.

#### Example 6

To determine the permanency of this additive treatment, one piece of cloth, treated as described in Example 3, was washed in hot Alconox solution, rinsed, and dried; another piece of treated cloth was dipped in perchloroethylene and dried, six times. Neither cloth showed any static activity, indicating that the additive was still retained on both pieces of cloth.

#### Example 7

A piece of cloth was dipped in a 1.0% solution of tri-methyldisoya ammonium phytate in isopropanol and then dried. The cloth showed no static activity in the tests described above. A Lucite rod, dipped in this solution and dried, also showed no static activity.

The foregoing test results demonstrate the remarkable properties of the synthetic textile materials treated with organic ammonium phytates.

In summary, the applicant has discovered that a class of materials, the ammonium phytates, have particular utility in promoting electrical conductivity in treating non-conductive solid materials, in particular textile fibers and fabrics. The preferred ammonium phytates are those oil-soluble aliphatic ammonium phytates with the tertiary ammonium phytates especially preferred, while mixed quaternary-tertiary ammonium phytates are particularly preferred additives. It will be understood that modification within the skill of those adept in the art may be made without departing from the scope of the invention.

What is claimed is:

1. A solid synthetic hydrophobic non-conductive material selected from the group consisting of fiber and cloth containing on its surface a minor amount sufficient to promote electrical conductivity of said material of an organic ammonium phytate consisting of a negatively charged phytate anion and 1 to 12 positively charged ammonium base cations wherein each of said cations consists of an ammonium nitrogen atom and 1 to 4 organic radicals bonded to said nitrogen atom by carbon-to-nitrogen bond, each of said organic radicals containing 1 to 30 carbon atoms.

2. A material as defined by claim 1, wherein said phytate contains 1 to 6 of said cations and wherein each of said cations has a carbon-to-nitrogen atomic ratio of greater than 2:1.

3. A material as defined by claim 1, wherein said organic radicals are aliphatic radicals.

4. A material as defined by claim 1, wherein said phytate is methyldisoya ammonium phytate.

5. A material as defined by claim 1, wherein said phytate is dimethyldioleyl ammonium phytate.

10

6. A process for reducing the tendency of solid synthetic hydrophobic non-conductive material selected from the group consisting of fiber and cloth to generate and accumulate electrical charges, which process comprises coating the surface of said material with a minor amount, sufficient to promote electrical conductivity, of an organic ammonium phytate consisting of a negatively charged phytate anion and 1 to 12 positively charged ammonium base cations wherein each of said cations consists of an ammonium nitrogen atom and 1 to 4 organic radicals bonded to said nitrogen atom by a carbon-to-nitrogen bond, each of said organic radicals containing 1 to 30 carbon atoms.

7. A process for reducing the tendency of solid synthetic hydrophobic non-conductive material selected from the group consisting of fiber and cloth to generate and accumulate electrical charges, which process comprises coating the surface of said material with a volatile liquid solvent containing dissolved therein about 0.1 to 10 wt. percent of the organic ammonium phytate consisting of a negatively charged phytate anion and 1 to 12 positively charged ammonium base cations wherein each of said cations consists of an ammonium nitrogen atom and 1 to 4 organic radicals bonded to said nitrogen atom by a carbon-to-nitrogen bond, each of said organic radicals containing 1 to 30 carbon atoms and subsequently evaporating said volatile liquid solvent to thereby coat said material with said phytate.

20

25

30

35

#### References Cited by the Examiner

##### UNITED STATES PATENTS

2,256,112 9/1941 Dickey et al. ---- 252—8.8 XR  
2,279,502 4/1942 Dickey et al. ----- 252—8.8

JULIUS GREENWALD, Primary Examiner.